

Patented Mar. 6, 1928.

1,661,879

# UNITED STATES PATENT OFFICE.

DENIS DE GÖNCZ, OF NORTH ADAMS, MASSACHUSETTS, ASSIGNOR TO ARNOLD PRINT WORKS, OF NORTH ADAMS, MASSACHUSETTS, A CORPORATION OF MASSACHUSETTS.

## TREATMENT OF CELLULOSIC MATERIALS.

No Drawing.

Application filed September 22, 1924. Serial No. 739,201.

This invention relates to the treatment of textiles and other constructions of cellulosic material, such as cotton, jute, linen, ramie, wood and other vegetable fibres, for example cotton yarns or cotton cloth; and to an improved textile product resulting from the treatment.

Heretofore constructions of these materials have been subjected to solvent or partially solvent and other chemical treatments for the purpose of reconstituting their texture by the development of cellulosic derivatives in a rearranged and improved physical condition as compared with the natural material, fibre, or texture.

The present process has for one of its objects to improve the steps of treatments of this category for economy of time and material, certainty of result, and an improved effect or final state of the product.

The practices of the prior art do not attain the effect gained by the present process, and are moreover in general characterized by difficulties in realization due to lack of stability or variable quality of the reagents necessarily employed. For example, a preferred solvent reagent of old use is an ammoniacal solution of copper, or "cuprammonium" so-called. Heretofore it has been customary, if not necessary, to use a solution containing caustic alkali, without which alkaline qualification the reagent is not certainly or sufficiently active upon the fibrous cellulose. But this fact has militated against the use of this reagent, because an alkaline ammoniacal solution of copper is prone to break down spontaneously, with separation of copper oxide. This has led to uncertainty of results and to necessity for frequent renewals of the solution, as well as to ineffective or damaging treatment of the cloth when the solution decomposes during a run of treatment.

Such treatments of vegetable-fibre fabrics have heretofore been characterized in groups roughly identifiable by their effects as those producing mercerized fabrics and those producing parchinentized fabrics, with some variations relating to the physical state of the surfaces of the fabric, such as the production of high silky glosses by mercerizing and stretching, of wrinkled or creped effects, or effects upon vegetable fibres resembling the texture of wool. The effect gained by the present invention is a trans-

formation or conversion of the component yarns to the natural effect of long-line linen, the product being cool to the touch, smooth, glossy, having a superficial transparent skin effect, slightly lessened flexibility, high absorption and permeability, improved tensile strength, and freedom from stray thin fibres or "fuzz". The most advantageous material for treatment in the case of textiles is cotton.

In the preferred practice, the material to be treated is made to carry a reagent substance in measured quantity entrained with the texture of the material into the presence of a cellulose solvent adapted to be activated by the presence of the said material-carried reagent in its solvent or other reactive capacity toward the cellulosic material.

For example, there will herein be described in detail, as one instance of this invention, the application of a measured dosage of an appropriate reagent to a sheet material to be treated. If the solvent is to be an ammoniacal solution of copper, a preferred reagent to be carried by or entrained with the material is an alkaline solution such as caustic soda, which may be supplied to the material in any convenient way for securing a uniform distribution, as by padding by dipping and squeezing (or partially drying, or both); or by treatment otherwise securing an even distribution on the surfaces and in the capillary spaces of the cloth or other material of the reagent or activating solution. But I am not to be understood as limiting this process to the treatment of every part of a web of material, since the treatment obviously may be applied locally if desired.

When this alkaline reagent is so applied, both a predetermined concentration of the reagent and a predetermined content of water and alkali in relation to the cellulosic volume or effective surface area of the material may easily be secured. This is the more readily attained when the concentration of the alkali when applied, as is recommended, be not greater than 19° Twaddell, (equivalent to 8.45% NaOH) and therefore insufficient in itself to cause any material chemical effect such as mercerizing at the normal temperatures and times of treatment other than adsorption upon the cellulosic contents of the alkaline contents.

When the material is prepared by associat-

ing with it an alkaline reagent in this manner, the capillary and adsorptive association of the material to be treated with the alkaline reagent prevents or inhibits the activating reagent from leaving the surfaces and capillary spaces of the fabric or material in a subsequent dipping bath. This is important, because while the reagent is necessary to activate the solvent, it is thus ensured that the solvent be not degraded by any substantial diffusion of the activating agent away from the material to be treated and into the solvent solution. This localizes the reaction at the surfaces and in the capillary spaces between the fibrous elements of the cloth; avoids activating, and thus promoting decomposition, of the treating solution in general; and has other advantages.

The amount of reagent capable of being entrained and carried by the material will of course vary with the material, with the particular reagent, with the concentration of the reagent, with the evaporative treatment, if any, resorted to decrease the water and increase the concentration prior to treatment in a wet state with the solvent proper; but in any case, I have discovered that when the material so carries a measured dosage of the activating reagent which primarily operates according to its chemical, physical or catalytic nature, into the presence of the solvent (for example, respectively, cotton cloth carrying caustic soda solution into the presence of ammoniacal copper solution), there ensues a three-part reaction participated in by the activating reagent, by the solvent solution, and by the nascent cellulosic surface, solution or colloid extension formed at the seat of the reaction. This reaction, whatever its true nature in a physical or chemical sense, is not only highly effective to produce the effect of linen on cloths of other vegetable fibres but the reaction proceeds with controllable regularity at practicable high speeds, and especially in the case of alkali-activated copper-ammonia solvent, results in high economy of solvent chemicals, the losses of the caustic and solvent baths being only those directly attributable to causing the improvement in the cellulosic material. I attribute the gains of solvent efficiency and regularity of action to the superior effect of a solvent in a state of being uniformly and locally activated by the entrained activating substance, as well as to the superior type of application to the cellular surfaces secured by confinement to and against them of the seat of chemical activity; and to the relatively large proportion of reactive cellulose in the presence of the entire active quantity of the reagent solution, thus effectively provided for.

Details of the treatment may be varied according to the material to be treated and the degree of conversion desired to be re-

alized. The weight or cellulosic mass-contents of the cloth to be treated, for example, to a degree indicates the concentration of the reagents, especially of the alkaline activating reagent, and the state of the material attained by previous usual treatments, such as bleaching or mercerizing treatments, may also be taken into consideration. One of the advantages of this treatment resides in the ease with which the previous state, weight, density (and in general, the reaction power) of the material treated may be compensated for, and in the consequent applicability of this process, with predetermined desirable results of a linenzizing finish, to cotton cloths and other materials of widely varying mass, texture and previous conditions of treatment.

The invention is well illustrated by reference to typical examples of practice as follows:

A relatively heavy continuous web of cotton (for example, of double-cloth suitable for vestings, collars or shirts) without previous treatment except scouring to make it absorbent, or bleaching when desirable, is continuously passed at a predetermined rate through a bath of a solution of caustic alkali in a suitable dipping and squeezing or other padding device; or the alkaline solution is otherwise suitably applied, in such a way as to effect a brief wetting contact with and entrainment of the solution on the surfaces and in the capillary spaces of the cloth. The web continues for a predetermined time of travel (insufficient in relation to the alkaline concentration for reaction of the solution with the cellulose in any chemical sense) and with or without evaporative conditioning of the entrained reagent, into prompt contact with a dipping or other applying bath of the solvent reagent, preferably "cuprammonium" as mentioned below. Here also the time of treatment, controlled by the length of the bath and the rate of passage of the web, is very brief. Thereafter the web is treated to neutralize, washed, stretched and dried.

In the instance given, a solution of commercial caustic soda of 19° Twaddell (1.095 sp. gr.) at normal room temperatures of 20° to 30° C. in contact with the fabric for six to eight seconds between first contact and the solvent bath, without substantial intermediate evaporation, is satisfactory. The alkaline entrainment in the fabric is well secured by passing under a dip roll in a trough vat of the solution, to emerge between squeeze rolls and immediately pass to a similar padding machine for the solvent treatment, the padding machines being conveniently close together, and the cloth traveling at the rate of thirty to forty yards per minute.

The solvent bath preferred in the given case contains forty pounds of copper sul-

phate and seven gallons of commercial strong ammonia water, made up to twenty-five gallons by added water. The solvent padding bath may, according to the dimensions of the bath and speed of the web, have an actual effective duration of from three to five seconds.

As the fabric leaves the squeeze rolls of the second or solvent padding machine, it is received on an ordinary lateral-stretching tentering frame, upon which the ammonia evaporates from the solvent, and the fabric is observed to be blue from the precipitated copper oxide of the reaction in the padding bath. During or after tentering, preferably after, the cloth is soured in dilute sulphuric acid, recommended to have a concentration of 6° Twaddell (1.03 sp. gr.), washed in copious water, and laundered, dried, ironed or calendered as may be desired.

The concentration of the caustic bath may be utilized for control of the effect, and should be lessened when the mass of the web is less, or when previous treatment, such as 25 yarn or piece mercerization, has increased susceptibility of its cellulose to solvent reactions. A plain muslin for example, under the conditions of treatment above indicated, is recommended to be padded with a caustic 30 solution of about 14° Twaddell (1.07 sp. gr.) concentration, and concentrations as low as 12° Twaddell may be advantageously employed when the previous condition of the web renders it highly sensitive.

35 For light fabrics, the ammoniacal copper solution may also be reduced in concentration; for example, to half the concentration above mentioned.

When I refer to padding the reagent substances into or upon the material to be treated, it will be understood that I do not necessarily refer to complete bibulous saturation. In many cases it is advantageous and desirable to limit the application of the 45 entrained reagent to one surface, or to a pattern. For these purposes, the padding treatment may be carried out by spraying, by printing, by stenciling or with the aid of resists applied to the webs superficially or 50 interstitially. However the application of the activating reagent is performed, it is preferable to remove any wet excess before contact with the solvent solution, in order to avoid degrading the solvent solution by 55 transfer to it of any free excess alkali. This process is thus in part characterized by the preliminary association of the cellulosic structure with the activating substance, and the subsequent contact of this association 60 with the solvent substance to be activated.

Whatever may be the mutual interaction between the cellulose, the alkali, and the cuprammonium, the ultimate effect indicates the reaction to be catalytic in character.

65 The cuprammonium solutions employed

when acting independently on cellulose are of such a degree of dilution as to be substantially inert; the alkaline solution is correspondingly ineffective alone, whereas the solvent effect of the tripartite group of cellulose, alkali and cuprammonium on its cellulose member is most pronounced and exceedingly rapid. It may be postulated that copper oxide is formed by reaction between the cuprammonium compound and the alkali, 70 and that the copper oxide, in a finely divided and nascent state, is a catalyst for the action of the contact film of the remaining substances in solution upon the cellulose. It will be observed that the recommended treatment places the tripartite group in necessary contact with the material to be treated throughout the possible seat of any reaction, and that the reagents are nowhere else in an active state. A constant effect on the material treated, uniformly distributed and invariable in degree of chemical activity, in accordance with the predetermined concentrations, temperatures and times, is thus 80 secured.

It is to be understood that the specific instances of practice of this process herein described are illustrative only of the principle of the invention, which is not limited to the species used for illustration. For example, it is obvious that other activating reagents or other solvent solutions may appropriately be substituted, and that the principle of the invention is independent of mere choice of materials to be treated or 90 reagents for the treatment, or concentration temperatures or times of reactions, so long as the material, the activating substance and the solvent substance are brought into association for the useful effects, or 100 any of them, gained by this invention.

Cellulosic materials, whether treated as fibrous stock or after making into yarns or into fabrics such as cotton cloth; and particularly the heavier grades of textiles, 110 such as sheeting, osnaburgs or collar cloth, treated in accordance with the invention, acquire a more lustrous surface and have more sheen. According to the degree of treatment, more or less of the fuzz is removed, and individual fibres tend slightly to agglomeration in bundles, to become rounder, without substantial loss of diameter, and the integuments of the fibres become less striated, smoother, stiffer and harder. Optically, the treated fibres are more polished and superficially more transparent. It will also be observed that the individual yarns, when the fabric is a woven or knit fabric, 115 are slightly stiffened, have a greater tensile strength, that there is little or no cementing tendency at points of contact between yarns, and that the permanently slightly hardened surfaces which result give the smooth, cooling sensation to the touch which is charac- 120

teristic of linen; and finally, that all of these properties thus imparted to the fibres are permanent, resisting both the action of normal wear and subsequent washings. The fabrics resulting are thus permanently and insolubly dressed in effect, as if very lightly starched, but, as may be shown by raveling, no paper-like adhesions between yarns result from the described degree of treatment of an organized textile, and the flexible and durably flexible character of the textile structure is decreased merely in degree, without any loss of the useful qualities expected of a cloth. The cloth may thus be repeatedly folded and machine-sewed without breakage or increased difficulty of sewing. The qualities gained by the treatment are positive and valuable accordingly.

If lighter grades of textile fabrics are subjected to the treatment, they obtain in addition to the above properties also a very marked degree of transparency. The degree and uniformity of treatment effected is entirely under the control of the operator. The treatment improves the commercial value and standardizes the quality of the products, permits continuous operation, and results in an important economy of reagents, as compared with other usual glossing or converting treatments, and produces a product in which the glossing effect does not involve the tensile elongation with substantial loss of diameter, of the fibres composing the fabric, as is the case with fabrics glossed by alkaline reaction with concomitant heavy stretching.

The term "natural cellulosic material" as used in the claims is intended to include the well known vegetable fibres such as cotton, jute, linen, ramie and wood, but to exclude esters of cellulose such as the well known artificial silks and the like.

I claim:

1. Process of treating natural cellulosic material of the character described which comprises applying to such material a solvent activating agent, and thereafter subjecting the material containing the activating agent to the superficial action of a cellulose solvent.

2. Process of treating natural cellulosic material of the character described which comprises wetting such material with a solvent activating solution, and thereafter subjecting the material containing the activating agent to the superficial action of a cellulose solvent.

3. Process of treating natural cellulosic material of the character described which comprises applying to such material a caustic alkali, and thereafter subjecting the material containing the caustic alkali to the superficial action of a cellulose solvent. 80

4. Process of treating natural cellulosic material of the character described which comprises applying to such material a caustic alkali, and thereafter subjecting the material containing the caustic alkali to the superficial action of a cuprammonium solution. 85

5. Process of treating natural cellulosic material of the character described which comprises wetting such material with a caustic alkali solution, and thereafter subjecting the material containing the caustic alkali to the superficial action of a cuprammonium solution. 75

6. Process of treating natural cellulosic material of the character described which comprises filling the interstitial spaces of the material with a caustic alkali solution, removing excess caustic alkali solution, and introducing the material containing the remainder of caustic alkali into a cuprammonium solution for superficial action thereon. 80

7. Process of treating natural cellulosic material of the character described which comprises treating such material with a caustic alkali solution of a strength incapable of chemically affecting the cellulosic material during the time of such treatment, and thereafter introducing the material containing the caustic alkali into a cuprammonium solution for superficial action thereon. 90

8. Process of treating natural cellulosic material of the character described which comprises filling the interstitial spaces of the material with a caustic alkali solution of not substantially greater than 19° Twaddell concentration, and thereafter subjecting the prepared material containing the caustic alkali for a limited period of time to the superficial solvent action of a cuprammonium solution. 100

9. Natural cellulosic material of the character described superficially modified by the physical action of caustic alkali activated cuprammonium. 105

Signed by me at North Adams, Massachusetts, this fourth day of September, 1924. 110

DENIS DE GÖNCZ.